

## UNITED STATES PATENT OFFICE

2,613,626

## METHOD OF COLD DRAWING SHEET METAL

Forrest Jerome Whitney, Jr., Wayne, Pa., assignor  
to Heintz Manufacturing Company, Philadelphia, Pa., a corporation of Pennsylvania

No Drawing. Application July 21, 1948,  
Serial No. 40,001

2 Claims. (Cl. 113—51)

1

This invention relates to a method of facilitating the drawing of metal sheets.

An object of the invention is to provide an improved method of cold working metal sheets which has the advantages of permitting faster operation of the metal working machinery, decreasing the number of imperfect articles made in the metal working process, and decreasing the number of delays occasioned by stoning the parts of the metal working machinery, such as dies and the like.

An example of the application of this invention is in the drawing of a metal tub by use of hardened steel dies, the final product having a diameter of around 25 inches and a depth of about 24 inches, and formed from a circular flat sheet of steel (for example of type A1S1 Specification C1008) having a gauge of approximately .062.

Before putting the steel sheets through the drawing operations, a quantity of sheets to be coated are first washed in an alkaline bath to accomplish degreasing, after which they are rinsed in cold running water. The blanks are thereafter immersed in a bath having the following chemical composition:

|                               | Grams per liter |
|-------------------------------|-----------------|
| Zinc                          | 11.0            |
| P <sub>2</sub> O <sub>5</sub> | 9 to 9.5        |
| NO <sub>3</sub>               | 18              |
| Na <sub>2</sub> O             | 1.5             |
| Ni                            | 0.1             |
| Cu                            | 0.03            |
| NaNO <sub>2</sub>             | 1 to 1.5        |

The above bath is preferably used at a pH of 2.8 to 2.9, and at a temperature of 20 to 25° C., with an immersion time of 3 to 5 minutes.

After treatment in the bath, the blanks are rinsed in cold running water and dried. The blanks after this treatment have a thin coating of zinc phosphate tightly adherent chemically to their surfaces.

After the phosphate coating operation, the coated blanks are put through three drawing operations, before each of which drawing operations the blanks are dipped or coated by swabbing, with a lubricant. Various types of lubricants are used, and among the most desirable are the following:

1. 1% sodium soap—99% water.
2. 2% sulphonated tallow—98% water, with enough sodium hydroxide to produce a pH value of 8.

2

3. 1% chlorinated paraffin, forming an emulsion with 2% sodium soap, using 97% water.

The lubricating solutions set forth above are used in conjunction with the following lubricants, one of which is a pigmented type of composition, and the other of which is non-pigmented, the two compositions following being used to adjust the lubricating conditions by addition to whichever of the three above-listed lubricants is being used.

## Non-pigmented

24% animal fatty acid (lard, oil, or degras)  
24% vegetable fatty acid (soy bean fatty acid)  
15 6% solid alkali (NaOH)  
10% chlorinated wax  
Balance water.

## Pigmented

20 24% animal fatty acid (lard, oil, or degras)  
24% vegetable fatty acid (soy bean fatty acid)  
6% solid alkali (NaOH)  
10% chlorinated wax  
20% pigment (talc, or inert clay)  
25 Balance water.

The two lubricants just described are used to adjust the lubricating conditions, the non-pigmented lubricant being used for adjusting the conditions of the first draw, while the pigmented type disclosed can be used only for the second and third drawing operations, since it is too slippery for the first draw and would permit the blank to slide between the blank holders without getting a sufficient cup formed for the subsequent operation.

In one test operation of the type just described, 80 of the coated blanks were run through the dies, and only one of the 80 showed any evidences of pick-up by the dies, and friction was reduced as much as 75%.

An astonishing and unexpected result followed the processing of the 80 phosphate coated blanks, in that the processing of the 80 blanks was followed with drawing of an additional 70 uncoated blanks, and only one additional metal score from pick-up was observed in the 70 additional blanks, showing that the beneficial results were carried over (apparently by the dies). The results from the processing of the uncoated blanks are made all the more unusual when it is considered that in the ordinary stamping of the uncoated blanks using the same lubricants, but without previ-

ously processing a series of coated blanks, pick-up occurred as frequently as every third or fourth draw, and caused bad scoring of the stampings. It was also necessary to stone the dies frequently under the previous practice because of the metal which the dies picked up from the blanks.

By using the new method and first running a series of coated blanks followed by a series of uncoated blanks, it is obvious that considerable savings in the use of the coating solution will be provided.

I claim:

1. In the cold deep drawing of steel sheets by means of dies, the steps of providing a thin chemically adherent coating of zinc phosphate on a 15 quantity of said sheets, applying to said quantity of sheets, a non-pigmented lubricant containing a high fatty acid radical which chemically reacts with said coating, cold deep drawing said quantity of sheets by the use of dies whereby 20 there is transferred from said sheets to said dies as the deep drawing is effected material which includes at least some of the phosphate coating material and some of the product of said reaction, applying to a smaller quantity of uncoated 25 steel sheets a non-pigmented lubricant of the same type as applied to the coated sheets, and cold deep drawing said second smaller quantity of sheets by the use of the same dies, the lubricants being selected from the group consisting of approximately one per cent sodium soap—ninety-nine per cent water; approximately two per cent sulphonated tallow—ninety-eight per

cent water, the pH of the lubricant being approximately 8; approximately one per cent chlorinated paraffin, forming an emulsion with approximately two per cent sodium soap, using approximately ninety-seven per cent water.

2. A process as defined in claim 1, the number of coated blanks being in the order of 80, and the number of uncoated blanks being in the order of 70.

FORREST JEROME WHITNEY, JR.

#### REFERENCES CITED

The following references are of record in the file of this patent:

#### UNITED STATES PATENTS

|           |      |               |
|-----------|------|---------------|
| Number    | Name | Date          |
| 2,326,387 | Mill | Aug. 10, 1943 |

#### OTHER REFERENCES

Journal of Physical Chemistry, vol. 36, 1932, pages 3108-3114.

Smith, Press Working of Metals, 1st ed., page 92, pub. 1896 by John Wiley & Sons, New York city.

Dies, Their Construction and Use, page 303, by Woodworth, published 1903 Norman W. Henley & Co., 132 Nassau Street, New York, New York.

30 Deep Drawing Qualities Improved by Phosphating, Stamping and Forming Section of Heat Treating and Forging, for June 1943.

American Machinist, Feb. 13, 1947, pages 117-128.